

# UNITED STATES PATENT OFFICE.

EUGEN ANDERWERT, HERMANN FRITZSCHE, AND HEINRICH SCHOBEL, OF BASEL,  
SWITZERLAND, ASSIGNORS TO SOCIETY OF CHEMICAL INDUSTRY IN BASLE, OF  
BASEL, SWITZERLAND.

## PROCESS FOR PRODUCING ON THE FIBERS NEW COPPER COMPOUNDS OF SUBSTANTIVE ORTHOXYAZO DYESTUFF.

1,276,307.

Specification of Letters Patent. Patented Aug. 20, 1918.

No Drawing.

Application filed November 4, 1915. Serial No. 59,579.

To all whom it may concern:

Be it known that we, EUGEN ANDERWERT, chemist, a citizen of the Swiss Republic, HERMANN FRITZSCHE, chemist, a citizen of the Swiss Republic, and HEINRICH SCHOBEL, chemist, a citizen of the Swiss Republic, all residents of Basel, Switzerland, have invented a Process for Producing on the Fibers New Copper Compounds of Substantive 10 Orthooxyazo Dyestuffs, of which the following is a full, clear, and exact specification.

In our application for a U. S. Letters Patent, Ser. No. 59580, filed November 4, 1915, we have described the production of new 15 copper compounds of substantive orthooxyazo dyestuffs, which can be fixed like the known substantive dyestuffs without mordant on the various textile fibers, yielding hereby tints of excellent fastness to light, 20 washing and alkali.

We have now found that the copper compounds of the same orthooxyazo dyestuffs can also be produced on the fibers, by treating for instance the dyeings obtained directly on the fiber with the substantive orthooxyazo dyestuffs described in the applications for United States Letters Patent Ser. No. 144244, filed January 24, 1917 (divisional application of Ser. No. 54403), Ser. 25 No. 144243, filed January 24, 1917 (divisional application of Ser. No. 54403), Ser. No. 54513, filed October 7, 1915, Ser. No. 164795, filed April 26, 1917 (divisional application of Ser. No. 54513) and in the U. S. 30 Letters Patent No. 1210751, dated January 1917, subsequently on the fiber with copper salts or by dyeing the fiber with the said orthooxyazo dyestuffs in a bath containing copper salts.

40 The new process is illustrated by the following examples:

Example 1: The monoazo dyestuff prepared from orthodiazoparacresolfonic acid and

bonate, the goods being introduced into the dyeing bath at a temperature of 40-50° C., 55 the bath heated to boiling and maintained in ebullition for  $\frac{1}{2}$  to 1 hour. The dyeing obtained is rinsed and treated subsequently for  $\frac{1}{2}$  hour at 60-70° C. in a bath containing 2 to 3% copper sulfate and 1-2% acetic acid. 60 Hereafter the goods are rinsed and dried. The resulting tint is identical with that obtained by dyeing with the copper compound of the same dyestuff without subsequent treatment.

Example 2: The monoazo dyestuff resulting from 4:2:1-nitrodiazophenol and



is dyed in the manner employed for substantive dyestuffs in a bath containing

2% dyestuff,  
1% crystallized copper sulfate,  
20% sodium sulfate and  
2% calcined soda,

the goods being introduced into this bath at a temperature of 40-50° C. and the bath heated to ebullition for  $\frac{1}{2}$  to 1 hour. Hereafter the goods are rinsed and dried. The obtained dyeing is identical with that obtained with the copper salt of the same monoazo dyestuff.

In an analogous manner can be produced on the fiber the various other copper compounds of orthooxyazo dyestuffs described in our application for a U. S. Letters Patent Serial No. 59580, filed November 4, 1915. All the dyeings obtained are characterized by an excellent fastness to light, alkali and washing.

What we claim is:

1. The described process for producing fast tints on animal or vegetable goods, which consists in forming the dye in presence of the goods by acting with a soluble copper salt on a substantive orthooxyazo-dyestuff derived from a 2:5:7-aminonaphthol sulfonic compound.

2. The described process for producing fast tints on animal or vegetable goods,



is dyed in the manner usually employed for substantive dyestuffs with 5 to 40% crystallized sodium sulfate and 1 to 5% sodium car-

which consists in first dyeing the goods in a bath formed by a solution of a substantive orthooxyazodyestuff derived from a 2:5:7-aminonaphtholsulfonic compound and treating afterward the thus obtained dyeing with a solution of a copper salt.

In witness whereof we have hereunto signed our names this 6th day of October,

1915, in the presence of two subscribing witnesses.

EUGEN ANDERWEERT.  
Dr. HERMANN FRITZSCHE.  
Dr. HEINRICH SCHOBEL.

Witnesses:

ARNOLD ZUBER,  
AMAND RITTER.